

## UNITED STATES PATENT OFFICE.

ANTHONY G. DE GOLYER, OF BROOKLYN, NEW YORK.

## ALLOY.

No Drawing.

Application filed November 16, 1922. Serial No. 601,393.

To all whom it may concern:

Be it known that I, ANTHONY G. DE GOLYER, a citizen of the United States, and a resident of the borough of Brooklyn, county 5 of Kings, city and State of New York, have invented certain new and useful Improvements in Alloys, of which the following is a specification.

This invention comprises a new alloy containing as essential components iron, chromium and boron, and which may contain additional elements, such as carbon, silicon, nickel, aluminum, manganese, tungsten or molybdenum; and distinguished from the heretofore known chromium alloys by its 10 composition, and by the possession of numerous combined improved and advantageous properties, such for example, as marked resistance to oxidation at high and 15 low temperatures, resistance to the action of many acids and alkalis, high tensile strength, and readiness with which it may be cast, machined, forged, rolled, drawn, stamped or otherwise worked.

Various chromium containing alloys have been previously proposed with the object of providing metallic products to meet special requirements, but the properties have usually been so restricted as to render the 20 alloys unsuitable for general commercial application, and the use of these has been further limited by reason of the high cost of essential components, metallurgical difficulties in production of the alloys, difficulties 25 in the manufacture or products therefrom, etc.

The present invention provides an alloy which possesses numerous improved resistant and other properties; its essential components 30 may be derived from inexpensive ores, by-products or other materials; it may be produced by means of one or more cheap and comparatively simple methods, and it can be readily and economically utilized for 35 the manufacture of many articles for diversified purposes; consequently, the present alloy has distinct advantages of improved properties, ease and economy of production of the alloy itself, and the manufacture 40 therefrom of castings, forgings, stampings, wire and other articles of general commercial utility.

I have found that by alloying or otherwise 45 intimately combining iron and chromium with a comparatively small amount of boron, e. g., 15 per cent or less of the weight

of the final alloy, I obtain products of a metallic character which not only possess materially improved resistant and other properties, as compared to heretofore known 50 alloys or metallic products, but in many instances possess advantageous qualities not found in such other alloys or products. For example, an alloy combining high tensile strength, resistance to oxidation, rusting, 55 corrosion, etc., over a wide range of temperature, resistance to the action of many metals and nonmetals, such as carbon, sulfur, etc., many organic and inorganic compounds, and which may be readily cast, machined, welded, forged, rolled, drawn, stamped or otherwise worked, contains chromium from 5 to 35 per cent, boron from 0.25 to 15 per cent and virtually all of the balance iron; or an alloy which possess many 60 of the above important qualities, but, in some instances, is not as readily machined, rolled, drawn or stamped, and has high electrical resistance, is particularly resistant to oxidation, corrosion, etc., at low and extremely high temperatures, as well as the 65 action of many alkalis and acids, either hot or cold, concentrated or dilute, contains chromium from 20 to 60 per cent, boron 0.25 to 15 per cent and virtually all of the balance iron.

The proportions of the component elements may thus be more or less varied, i. e., the chromium content may be between 5 and 60 per cent and the boron content between 70 0.25 and 15 per cent with the iron varying accordingly; and one or more of the essential elements may be partially replaced by one or more additional elements. Therefore, the proportions of the elements in the alloy 75 may be determined, to a greater or less extent, by the requirements of any particular application, conditions of economy, etc.

Boron appears to be essential in many instances, and always highly advantageous for 80 imparting to the present alloy various definite properties and characteristics, such for example, as increased tensile strength, marked resistance to oxidation, rusting, scaling, burning, etc., at low and high temperatures, resistance to the corrosive or other action of many acids, alkalis, gases, molten 85 metals and metallic and non-metallic compounds. The presence of boron tends to insure the production of sound and homogeneous 90 ingots and castings; and such boron containing alloys may be cast, forged, ma-

chined, rolled, drawn, stamped or otherwise worked more satisfactorily and economically than alloys which contain chromium, but not boron. The boron may be present in this 5 alloy as boride of chromium, boride of iron, or in some other form.

Carbon is frequently present in the alloy of this invention, and while I may prefer to use an alloy which is free of, or does not 10 contain carbon in excess of 0.25 per cent, in some instances the alloy may contain as much as 1.50 per cent carbon without any 15 of the desired properties being adversely affected. Carbon may be present in combination with one or more metals or metalloids, or in uncombined or graphitic form, and in general it may be regarded as an impurity incidental to manufacture, as its presence does not appear to be of any particular 20 advantage, and may frequently be of disadvantage.

Silicon may be present in varying amounts, and while I usually prefer an alloy entirely free, or containing less than 1 25 per cent of silicon, in some instances it may be of advantage to have the silicon content between 1 and 15 per cent. The silicon may be present in combination with one or 30 more metals or metalloids, or in some other form.

The alloys of this invention may also contain sulfur, phosphorus, etc., usually as impurities incidental to manufacture, and the amount of such impurities should preferably be low, i. e., less than 0.50 per cent.

It will therefore be understood that the alloy of this invention may contain small amounts, e. g., 1 per cent or less, of one or more metals or metalloids in the nature 40 of impurities incidental to manufacture.

The alloy consists predominantly of iron and chromium, each of which exists in appreciable amounts; and boron, of course, in appreciable amounts up to 15% is an essential component of the alloy of this 45 invention. However, other metals or metalloids may be desired in the alloy for the purpose of giving it special characteristics or properties for special uses.

50 In some instances it may be of advantage to use as components of the present alloy, in addition to iron, chromium and boron, varying percentages of one or more metals or metalloids, such as aluminum, beryllium, calcium, cobalt, copper, magnesium, manganese, molybdenum, nickel, silicon, titanium, tungsten, uranium, vanadium or zirconium. Such components may be present in amounts between 0.10 and 60 per cent, 55 depending largely upon the character of the elements added and the properties desired in the final alloy. Thus, as a means of increasing tensile strength, malleability, 60 resistant properties, degree of hardness, melting point, electrical resistance, or for 65

other purposes, I may use one or more additional elements, such for example, as from 0.10 to 20 per cent manganese, molybdenum, aluminum, silicon, uranium, vanadium or zirconium; or from 0.50 to 60 per 70 cent nickel or cobalt; or from 0.50 to 35 per cent tungsten.

Products manufactured from the alloy of this invention thus combine numerous valuable and improved properties, and can be 75 used to advantage for many purposes, such for illustration, as:

Castings, forgings and other manufactured articles subjected to high temperatures; the action of carbon, alkalis, salts, 80 many acids, gases containing sulfur, etc., and sudden or intermittent cooling; such as carbonizing and annealing boxes or containers; melting pots for lead, copper, type metals, other metals or alloys, cyanides, nitrates, hydroxides, carbonates, sulfates, salts, etc., valves and other parts for internal combustion and other types of engines and motors; parts for furnaces, ovens, kilns, driers, stoves, etc., such as doors, 85 grates, supports, rails, rakes, automatic stoker parts, chains, links, tubes, etc.; chemical plant equipment, such as valves, pipe, tanks, pumps, etc., for handling sulfuric, acetic and other acids, sodium or 90 potassium hydroxide, sodium chloride, sodium or potassium cyanide, etc.; equipment for brewing, distilling, manufacture of food products, soap, etc.; ladles, slag pots, rolls, molds, dies, piercing tips, etc., for the working of metals, glass, etc.; retorts and other equipment for the refining of petroleum, 95 gas producers, metallurgical roasting furnaces, etc.; die casting molds for non-metallic compounds and vulcanizing equipment. 100

Castings, forgings, etc., for railroad and ship equipment and fittings, automobile wheels, bodies, etc.; dairy equipment, milk cans, etc.; laundry equipment; canning and packing house equipment; mining and metallurgical machinery, crushers, rolls, ball mills, stamps, etc.; structural members and other equipment for buildings, bridges, 110 radio and power transmission towers, roofs, etc.; cutting and grinding tools, abrasives; hardware, screens, filters, etc., steam and water fittings, plumbing; cutlery and other articles, such as rustless and stainless knives, forks, spoons, etc.; culinary utensils of all kinds; wire fencing; sporting goods, guns, golf clubs, etc.; tools and instruments of precision. 115

In the form of wire, strips, rods, ribbon, etc., as the heating element in electrical resistance furnaces, ovens, stoves, heaters, 120 irons and other equipment.

Alloys of this invention, in the form of semi-finished or finished articles of manufacture may be annealed or otherwise heat treated for the purpose of improving or im- 130

parting thereto any qualities or characteristics, e. g., such as increasing the tensile strength, ductility, malleability, etc., and such semi-finished or finished articles may be ground, polished, buffed or otherwise treated for the purpose of making the products more resistant to oxidation, rusting, corrosion, etc.

The herein described alloys may be produced by a number of methods, such for example, as by melting together preformed iron, chromium and boron in predetermined proportions; by adding boron or a boron containing compound, such as boron and calcium, boron and chromium, boron and iron, boron and nickel, boron and aluminum, etc., to a bath containing iron and chromium; or by the more or less simultaneous reduction of predetermined amounts of oxygen or other compounds of iron, chromium and boron.

I do not claim herein any of the improved metallurgical processes for the production of the alloys of the present invention, as these form the subject matter of additional applications.

Scrap or by-products resulting from the manufacture or industrial application of the alloys of this invention may be recovered by remelting, or other suitable means.

It will be evident that the present invention provides alloys possessing numerous improved and advantageous properties, and that the alloys may be composed principally of iron, chromium and boron in varying proportions and be entirely or substantially free of impurities; or they may advantageously contain varying amounts of one or more other metals or metalloids alloyed therewith.

It will further be evident that the improved alloys may be used for castings, forgings and other articles of manufacture, and that such products may be utilized for many different applications or purposes, and therefore I do not wish to be confined in the use of the improved alloys to any specific application or product.

I claim:

1. An alloy comprising chromium 5 to 35%; boron in appreciable amounts up to 15%; carbon in appreciable amounts up to 1.50%, the balance being principally iron. 50
2. An alloy comprising chromium 5 to 35%; boron in appreciable amounts up to 15%; the balance being principally iron. 55
3. An alloy comprising chromium 20 to 60%; boron; in appreciable amounts up to 15%; carbon in appreciable amounts up to 1.50%; the balance being principally iron. 60
4. An alloy comprising chromium 5 to 60%; boron in appreciable amounts up to 1.5%; carbon in appreciable amounts up to 1.5%; the balance being principally iron. 65
5. An alloy comprising chromium 20 to 60%; boron in appreciable amounts up to 15%; the balance being principally iron.
6. An alloy comprising chromium 5 to 60%; boron in appreciable amounts up to 15%; the balance being principally iron. 70
7. An alloy comprising chromium 5 to 60%; boron in appreciable amounts up to 15%; carbon in appreciable amounts up to 1.5%; calcium, tungsten, molybdenum, silicon, aluminum, manganese, nickel, cobalt, vanadium, titanium, uranium, and zirconium in appreciable amounts up to 25%; the remainder being principally iron. 75
8. An alloy comprising chromium 5 to 60%; boron in appreciable amounts up to 15%; calcium, tungsten, molybdenum, silicon, aluminum, manganese, nickel, cobalt, vanadium, titanium, uranium, and zirconium in appreciable amounts up to 25%; the remainder being principally iron. 80
9. An alloy comprising chromium 5 to 60%; boron in appreciable amounts up to 15%; tungsten in appreciable amounts up to 30%; carbon in appreciable amounts up to 1.5%; the balance being principally iron. 85
10. An alloy comprising chromium 5 to 60%; boron in appreciable amounts up to 15%; nickel in appreciable amounts up to 30%; carbon in appreciable amounts up to 1.5%; the balance being principally iron. 90

ANTHONY G. DE GOLYER.